

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## CONSTRUCTION MATERIAL

No Drawing.

Application filed March 25, 1925. Serial No. 18,328.

This application contains subject matter disclosed in my applications Serial No. 437,- 622, filed January 15, 1921 and Serial No. 472,319, filed May 25, 1921.

5 Heretofore it has been the practice to mix fibrous material and asphalt, the fibrous material being as a rule such material as is readily penetrated by the asphalt, into a mass formation, which upon pressure readily elongates and in warm weather the expansion joint becomes very limber and flexible, thus difficult to manage.

10 My invention relates to a structure and process which if followed creates the structure described herein.

I have found that in utilizing mixing machines for incorporating stiff masses into the ductile substance which may be asphalt or any other compound having a ductile nature, 20 and by incorporating said materials in considerable proportion, and later passing said batch or body of mixed material between belts, which draw in one direction, which machines have also been previously described, 25 and are known to the art, that by reason of feeding a stiff and large mass to said machine, the fibrous matter or particles incorporated therein are made to arrange themselves in a laminated formation between layers of water- 30 proof binding material, most of the fibrous matter stringing itself and forming itself so as to lay in one direction, making a series of laminated layers alternating with each other on the order of a shale-like structure which 35 build up an internal structure in a body of ductile material.

I use preferably strips of saturated felt or scrap roofing strips preferably  $\frac{1}{2}$ " x 2" or any other suitable size, or other roofing material or fibre which may be in the nature of a waste product or a specially treated product, and for this purpose anything having a sufficient body to resist breakage in the mixing will answer for the structural reinforcement.

40 45 The binding material may be a blown asphalt or rubber, resin compound or any like combination preferably of a water-resisting nature, and the percentage of such ductile matter would approximate 70% to approximately 25 to 30% of the scrap or fibrous ma-

terial. The batch is generally mixed at a melting point in which the material is not in excess of 300°, as better results will be obtained by mixing at the lower temperatures, although fairly good results can be obtained by mixing at the higher temperatures.

55 The basis in forming my invention consists of a batch or mixture as described and in drawing the batch between belts and between pressure rolls which cause the asphalt to align itself and in doing so pull the fibre or strips in one direction, making a board having the grain in one direction and a cross section the same as lumber. This material is preferably rolled in thin sheets and may 60 be used for roofing, expansion joints in road construction, siding or any other suitable material in the construction line.

65 The fibrous material may be saturated or unsaturated or may be treated with any asphaltic or other suitable material which may increase its strength, the main object being to secure a laminated shale-like structure with the fibre or strips running in the direction of the pull of the belts or amalgamated 70 in a manner to form strength in the ductile material.

75 To reproduce the product described I proceed by first melting the ductile material, blown asphalt as an example, so as to reduce the same to a liquid consistency. Unless the asphalt was melted in a mixer I 80 would, of course, have to transfer it to a mechanical mixer, preferably one that has heating facilities, so as to retain the asphalt 85 at the desired liquid consistency.

90 In starting the mixer up with a predetermined quantity of the asphalt collected in the same I proceed to add successive quantities of the filling material until the desired ratio with respect to the asphalt had been incorporated. The addition of the filling material of course thickens the asphalt. After the mixing had been carried out to a 95 point where a thorough mix has been realized, I remove the mass from the mixer and introduce it to sheet forming apparatus, such as the belts referred to, where it is reduced into the form of sheets. The belts, as explained, set up a flow in the mass which 100

will align the pieces of filling material and cause them to lie in the direction of the feed of the asphalt thru the belts, thus developing the laminated, shale-like structure referred to. In using rubber or a resin compound the same may be added to the asphalt prior to the incorporation of the filler.

I claim:

- 10 1. Constructional material comprising a sheet of waterproof ductile material having a filler mixed therewith in the form of flat scraps of roofing material separated from each other by thicknesses of the ductile material.
- 15 2. Constructional material comprising a sheet of waterproof ductile material having a filler mixed therewith in the form of flat strips of felt separated from each other by thicknesses of the ductile material.
- 20 3. Constructional material comprising a sheet of rubber and a resin compound having a filler mixed therewith in the form of roofing scrap, separated from each other by thicknesses of the compound.
- 25 4. Constructional material comprising a sheet of rubber and asphalt compound having a filler mixed therewith in the form of laminated flakes of felt, separated from each other by thicknesses of the compound.
- 30 5. Constructional material comprising a sheet of rubber, asphalt and resin compound, having a filler mixed therewith in the form of laminated flakes of felt separated from each other by thicknesses of the compound.
- 35 6. Constructional material comprising a sheet of waterproof, ductile binder having mixed therein flat and relatively thin strips of fibrous roofing scrap.

ALBERT C. FISCHER.

40

45

50

55

60

65